

## 1

3,476,850

**LOW ELONGATION SET SPANDEX FILAMENTS  
AND PROCESS FOR THE PREPARATION  
THEREOF**

Kanji Matsubayashi and Hiroyuki Segawa, Kurashiki-shi, Japan, assignors to Kurashiki Rayon Co., Ltd., Kurashiki-shi, Okayama-ken, Japan, a corporation of Japan  
No Drawing. Filed Apr. 3, 1967, Ser. No. 627,667  
Claims priority, application Japan, Apr. 5, 1966,

41/21,656

Int. Cl. D01f 7/00; D02j 1/22

U.S. Cl. 264—205

4 Claims

**ABSTRACT OF THE DISCLOSURE**

Process for the preparation of spandex filaments of temporarily lowered elongation characterized in that spun filaments of a polyurethane elastic polymer by dry spinning are subjected to a heat treatment to reduce the solvent content remaining therein to no more than 0.5% by weight, the obtained filaments being further subjected to drawing, heat setting, cooling and shrinking operations.

This invention relates to a process for the preparation of spandex filaments of which elongation is temporarily lowered.

Heretofore, spandex or rubber filaments offered great difficulty for proper tension control during their post-treatments such as spinning, knitting and weaving because of their very high elongation of above 300%, normally even higher than 500%.

As a means to overcome this difficulty, a process was proposed in which elastic fibers are coated with a water-soluble polymer such as polyvinyl alcohol and set, but satisfactory setting effect cannot be thereby achieved. There is still another process proposed which comprises mix-spinning water-soluble polyvinyl alcohol or a non-elastic polymer which is soluble in organic solvents with an elastic polymer, drawing the resultant mixed fiber to impart thereto a fixed elongation, making therefrom such products as knit or woven goods or semi-products as filaments or mixed yarn by suitable post-treatments and thereafter dissolving off the non-elastic polymer so that the products should exhibit the elastic characteristics inherent in the elastic fiber. However, this process has its drawbacks such as complicated spinning step, difficulty for satisfactorily complete removal of the non-elastic polymer in the dissolving step, deformation caused in the section of the elastic fiber after removal of the non-elastic polymer, and high production cost.

Previously we proposed a process effective for imparting a low elongation, by drawing the filaments containing more than 0.5 wt. percent of the solvent still remaining therein immediately following the spinning step. Although low elongation set spandex filaments are obtained by the above drawing treatment of the solvent-containing spun filaments in accordance with the above process, permanent deformation is conspicuous in the resultant filaments which do not entirely recover their characteristics as the high elongation spandex filaments possessed before the drawing, at the stage of shrinking of the products prepared from the filaments such as yarn, knit or woven goods. For example, a polyurethane spun filament containing 1.0 wt. percent of dimethylformamide having an elongation of 430% was given a lower elongation of 110% when drawn by 3 times, but when the same was subsequently treated for 10 minutes in 100° C. water free of tension, its elongation became 265%, thus failing to regain the elongation possessed before the drawing step. Again when the spun filaments contain a large volume of the solvent, high temperature drawing tends

## 2

to cause filament breakage, while relatively low temperature drawing makes the drawing control insufficient when the drawing speed is high.

We therefore engaged in further researches to find that polyurethane spandex shows behaviours close to one point drawing different from rubber, the tendency being particularly conspicuous in the polyurethanes prepared with a low molecular diol serving as the chain extender, compared with the polyurethanes prepared with other chain extenders such as hydrazin, diamine or water. Furthermore it is found that the tendency is enhanced under elevated temperatures. And, according to the invention the said polyurethane showing the behaviours of one point drawing for which a low molecular diol is used as the chain extender is found to possess the property to form far better spandex filaments of temporarily lowered elongation intended by the invention, compared with such polyurethanes prepared with other chain extenders, e.g., water, diamine and hydrazin. Still in addition we found substantially complete removal of solvent from the polyurethane filaments before the drawing to be highly effective for the preparation of the spandex filaments of which elongation is temporarily lowered. Those discoveries led us to the present invention.

Accordingly the object of the invention resides in the preparation of the spandex filaments of excellent properties and furthermore having an elongation temporarily lowered to around 100%, by the process which comprises dry spinning a spinning solution of a polyurethane elastic polymer in a heated spinning column and preparing spandex filaments having high elongation similarly to conventional spandex filaments, substantially completely drying the solvent in the subsequent drying step, drawing the filaments, heat setting the spandex filaments under tension, further cooling the same to at least below 50° C. and thereafter shrinking the same by 5–15% of the original length.

In the invention, a particular care should be taken to secure a sufficient drying until the amount of the solvent remaining in the filaments after spinning and before drying is reduced to no more than 0.5 wt. percent to the filaments. Because, in case filaments containing more than 0.5 wt. percent of solvent are subjected to drawing, heat setting, cooling and thermal shrinking in accordance with the invention, admittedly fibers having an elongation of around 100% are obtained which, however, fail to perform sufficient shrinkage during the heat treatment at around 100° C. free of tension and consequently cannot regain the high elongation possessed before the drawing. For instance, a dimethylformamide solution of a polyurethane elastic polymer prepared from the three components of polyethylene propylene adipate (ethylene:propylene copolymerization=9:1), 4,4'-diphenylmethane diisocyanate and ethylene glycol (molar ratio=1.0:5.0:4.0) was dry-spun, and the resultant filaments having an elongation of 435% and a dimethylformamide content of 0.8 wt. percent were drawn, heat set, cooled and thermally shrunk in accordance with the process of this invention. Thus prepared fiber had an elongation of 118%, but when treated in 100° C. water for 10 minutes free of tension, it came to have an elongation of only 277%.

The temperature employed for drying of the solvent in accordance with the invention should be above boiling point of the solvent but no higher than 200° C. With the drying temperature below boiling point of the solvent, drying efficiency is poor, and such high temperatures exceeding 200° C. should also be avoided because at the temperatures close to the melting point of the filaments fusion among the mono-filaments tends to take place.

Again the drawing temperature in accordance with the invention should be within the range of 80–150° C., preferably 120–150° C. Because, at temperatures below 80°

C. the desired high speed drawing is inoperable, while at above 150° C. ideal one point drawing cannot be achieved, causing an uneven drawing effect. Furthermore, the draw ratio should be 2-6 times the original length of the filaments, for the reason that at a draw ratio less than 2 fibers of sufficiently lowered elongation cannot be obtained even after the heat setting, cooling and thermal shrinkage in accordance with the invention, and on the other hand with high draw ratios exceeding 6 and approaching the breaking point of the fibers, degradation in strength properties of the fibers is invited.

The heat setting temperature should range 150-200° C., preferably 160-180° C. Heat setting at below 150° C. could achieve the intended effect with prolonged setting time when the drawing temperature was below the said level, but such is not an industrially recommendable procedure. Once again temperatures exceeding 200° C. being close to the melting point of the filaments, setting at such high temperatures tends to cause objectionable fusion among the monofilaments even within a short time.

Normally the heat setting in the order of 2-15 seconds can achieve the intended result.

Again in accordance with the invention it is necessary to cool the heat set filaments at below 50° C., preferably to room temperature, to stabilize the shrinking portions of the filaments formed when they are freed from tension, which were not heat set in the preceding step, and thereafter to shrink the filaments by 5-15% of the original length thereof. The purpose of this last shrinking is to prevent the occurrence of non-uniformity in properties of the products such as non-uniform denier and strength distribution when the elastic fibers of the invention are, for example, mix-spun, combined or subjected to other treatments with non-elastic fibers, such inuniformities being caused by the shrinkable portions present in the elastic fibers. In this shrinking step, the shrinkage should be by 5-15% of the original filament length. With a shrinkage less than 5%, substantial shrinking effect is hardly obtainable although the purpose of temporary fixing of elongation may be achieved. Whereas, when it exceeds 15%, the treated filaments are given an elongation of above about 150% to render the temporary fixing of the elongation ineffective. The shrinking can be performed between two rollers of different rotation speed at room temperature or with heating. In case of heating, incidentally, still the temperatures of the rollers should be at below 50° C.

Thus in accordance with the invention there is an advantage that even when the drying, drawing, heat setting, cooling and shrinking steps are performed as a continuous series to the spinning step, still low elongation set spandex filaments of uniform quality and even elongation distribution as desired can be obtained.

The spandex filaments thus prepared having an elongation of around 100-120% and a tenacity of about 2.0-4.0 g./d. of the invention can be mix-spun, knit or woven with non-elastic fibers such as nylon and polyester using ordinary equipments for mix-spining, knitting or weaving, without requiring the complicated tension control machine employed with conventional spandex filaments processing. Thus obtained knit or woven goods as they are fail to exhibit sufficient elasticity due to the low elongation of the material spandex filaments, but upon allowing the products to sufficiently shrink by heating the same to above 90° C., preferably about 100-150° C., so that the spandex filaments may regain the high elongation originally possessed before the drawing and heat setting, products having excellent elastic characteristics are obtained.

The invention now will be explained as to an embodiment for working the invention.

The spinning solution of a polyurethane elastic polymer of the invention is fed into a spinning head by means of a gear pump and extruded into a heated spinning column through which a heated gas is passed, from a nozzle in

the spinning head. The filaments whereby formed contain about 4 wt. percent to the spun filaments of the solvent remaining therein when they leave the spinning column. The same are then led to godet rollers via oiling rollers and guides. The filaments thus containing about 4 wt. percent of the solvent are further well dried by means of heated Nelson rollers for drying to have the remaining solvent content reduced to no higher than 0.5 wt. percent. Thereafter the filaments are drawn between two rollers and heat set by means of heat setting Nelson rollers, followed by cooling by means of cooling rollers which are not heated but maintained at room temperature. The filaments are then slightly shrunk between two rollers and taken up onto a take-up machine.

As the polyurethane elastic polymers useful for the invention, block copolymers consisting of the following three components are employed: polymer diol of melting point no higher than 60° C. and molecular weight ranging 500-5,000, preferably 800-3,000, and having terminal hydroxyl radicals; aromatic diisocyanate; and low molecular diol of molecular weight ranging 50-200.

Specific examples of such polymer diol having terminal hydroxyl radicals include: polyethylene adipate, polyethylene propylene adipate, polybutylene adipate, polyhexamethylene adipate, polyethylene butylene adipate, polycaprolactam, polytetramethylene glycol, polypropylene glycol and polyethylene glycol.

As the aromatic diisocyanate, 4,4'-diphenylmethane diisocyanate, 3,3',5,5'-tetramethylidiphenylmethane-4,4'-diisocyanate, 2,4-toluene diisocyanate, 2,6-toluene diisocyanate and the like are employed.

While any diol having a molecular weight ranging 50-200 may be used as the chain extender, for example ethylene glycol, 1,4-butanediol, 1,6-hexanediol and the like are preferred.

The polyurethane elastic polymers contemplated in the invention are prepared from aforesaid three components, viz., high molecular polymer diol, aromatic diisocyanate and low molecular diol. They may be prepared in accordance with accepted practices. One of the known means for their preparation comprises reacting a polymer diol with an aromatic diisocyanate to form a prepolymer in which the terminal radicals of the polymer diol are isocyanate group, adding thereto each suitable amount of the aromatic diisocyanate and a low molecular diol to form a polyurethane block polymer. It is also possible to mix the three components from the start and react them. Furthermore, those reactions may be performed in a solvent such as dimethylformamide, dimethylsulfamide or methyl isobutyl ketone, in the presence of a catalyst.

Those polyurethane elastic polymers are the optimum starting materials for the spandex filaments of temporarily lowered elongation.

As the spinning solutions, those prepared by dissolving the above polyurethane elastic polymers in suitable solvents such as dimethylformamide, dimethylacetamide, tetrahydrofuran and dimethylsulfoxide are used.

Hereinafter the invention will be explained with reference to the working examples.

#### EXAMPLE 1

The three components: polyethylene propylene adipate (ethylene:propylene copolymerization ratio=9:1) having a molecular weight of 2,000 and terminal hydroxyl radicals; 4,4'-diphenylmethane diisocyanate; and ethylene glycol were mixed at the molar ratio of 1.0:5.0:4.0, and the mixture was reacted in methyl isobutyl ketone at 100° C. for 4 hours in the presence of dibutyl tin dilaurate as the catalyst. After completion of the reaction, methyl isobutyl ketone was removed from the system by vacuum drying, and whereupon powdery polyurethane elastic polymer was obtained. To the same polymer a composition consisting of 2.0 wt. percent to the polymer of TiO<sub>2</sub>, 2.0 wt. percent of 4,4'-butylidene bis(3-methyl-6-tertiary butyl phenol), 0.5 wt. percent of acetic anhydride and 0.5

wt. percent of  $\beta$ -(lauryl thio-) ethyl alcohol was added, and the system was dissolved in dimethylformamide to be made into a spinning solution of 30% concentration. The solution was fed, after debubbling, into a spinning head heated to 100° C. under an elevated pressure, and extruded through a nozzle having 0.2 mm.  $\phi \times 10$  holes into a spinning column through which heated nitrogen was passed at the rate of 2 m.<sup>3</sup>/hr. (calculated as 30° C.). The spinning column was maintained at 180° C. in the vicinity of the nozzle, 300° C. at the top and 200° C., at the middle and lower portions.

The filaments thus spun had a remaining solvent content of about 5.0 wt. percent to the weight of the filaments containing the solvent immediately after they left the spinning column. Continuously to the spinning step, the filaments were dried for 5 seconds on Nelson rollers heated to 170° C. and driven at the rate of 350 m./min. Whereupon the solvent content of the filaments was reduced to 0.31 wt. percent.

Continuously to the above drying, the filaments were drawn by 3.5 times at 150° C., and heat set for 1.5 seconds on heat setting rollers heated to 170° C. and driven at the rate of 1,225 m./min. and for 2.0 seconds on heat setting rollers heated to 180° C., followed by cooling for 1.2 seconds on cooling rollers driven at the rate of 1,225 m./min. Then the filaments were shrunk by 10% by making the speed of the take-up roller (15° C.) 1,100 m./min. Filament breakage scarcely took place during the operation over tens of hours, and drawing control was excellently maintained.

The properties of the spandex filaments obtained thus in accordance with the subject invention are given in Table 1 below, from which it can be understood that the product is characterized by its low elongation, high tenacity, high Young's modulus and surprisingly great elasticity compared with conventional spandex filaments. Also from Table 1 it can be understood that the low elongation set spandex filaments return to the conventional spandex filaments of low tenacity and high elongation as they were before the drawing and heat setting steps, when subjected to a shrinking treatment in hot water.

TABLE 1

| Property                                                                | Spandex filaments of this invention | The same sample when shrunk in 100° C. water for 15 minutes free of tension |
|-------------------------------------------------------------------------|-------------------------------------|-----------------------------------------------------------------------------|
| Denier (d.)                                                             | 42                                  | 79                                                                          |
| Tenacity (g./d.)                                                        | 2.81                                | 1.38                                                                        |
| Elongation (Percent)                                                    | 105                                 | 377                                                                         |
| Young's modulus: tenacity at 10% elongation (g./d.)                     | 0.14                                | 0.04                                                                        |
| Elastic recovery after 50% elongation (Percent)                         | 102                                 | 96                                                                          |
| Shrinkage in 100° C. water (Percent)                                    | 54.0                                | 2.3                                                                         |
| Shrinkage after one month standing in air at room temperature (Percent) | 7.2                                 | 0.2                                                                         |

and could not recover the high elongation after the shrinking treatment.

Again frequent filament breakage was observed during the drawing, and even when the drawing temperature was gradually lowered, the drawing control or stability was much inferior compared with the case of the invention.

TABLE 2

| Property                                                                | Sample drawn with 3.0 wt. percent solvent content and heat set, cooled and shrunk | The same sample when shrunk in 100° C. water for 15 minutes free of tension |
|-------------------------------------------------------------------------|-----------------------------------------------------------------------------------|-----------------------------------------------------------------------------|
| Denier (d.)                                                             | 45                                                                                | 77                                                                          |
| Tenacity (g./d.)                                                        | 2.57                                                                              | 1.65                                                                        |
| Elongation (Percent)                                                    | 108                                                                               | 257                                                                         |
| Young's modulus: tenacity at 10% elongation (g./d.)                     | 0.10                                                                              | 0.05                                                                        |
| Elastic recovery after 50% elongation (Percent)                         | 99                                                                                | 93                                                                          |
| Shrinkage in 100° C. water (Percent)                                    | 43.2                                                                              | 1.1                                                                         |
| Shrinkage after one month standing in air at room temperature (Percent) | 6.6                                                                               | 0.1                                                                         |

Now the properties of a woven good prepared from the spandex filaments obtained in above Example 1 will be explained.

A fabric sample was prepared from mixed yarn consisting of wool 70% and polyester 30% as the warp (42, S) and the same mixed yarn with the spandex filaments of Example 1 as the weft. The spandex filament was used at the ratio of one thread to 3 strands of the mixed yarn. The weaving was well operable employing a conventional weaving machine, without using a special shuttle.

The fabric was pre-designed to have a spandex filament content of 3%, and a width of 2 m. The fabric showed little elasticity as woven, but when subjected to a series of post-treatments comprising relaxation in hot water to reduce the width to 1.5 m., drying to reduce it to 1.4 m., surface finishing by press treatment for 30 minutes in 120° C. steam, heat setting for 60 seconds in 180° C. dry heat to achieve dimensional stability and dyeing step free of tension, an elastic woven fabric of even surface was obtained.

Thus the elastic fabric in which the spandex filaments of the invention were used showed an elasticity of 30% and an elastic recovery of 94% when elongated by 20%. In contrast, the fabric prepared in the similar manner except using the spandex filaments containing 3.0 wt. percent of the solvent showed in an elasticity of only 22%.

#### EXAMPLES 2-4

Example 1 was repeated except that the heat setting conditions were varied each time. The properties of the resultant spandex filaments are given in Table 3.

TABLE 3

| Heat setting condition | Properties               |                            |             |                  |                      |                                                     |                                      |                                                                         |                                                                                                           |
|------------------------|--------------------------|----------------------------|-------------|------------------|----------------------|-----------------------------------------------------|--------------------------------------|-------------------------------------------------------------------------|-----------------------------------------------------------------------------------------------------------|
|                        | Heat setting temp. (°C.) | Heat setting time (second) | Denier (d.) | Tenacity (g./d.) | Elongation (percent) | Young's modulus: tenacity at 10% elongation (g./d.) | Shrinkage in 100° C. water (percent) | Shrinkage after one month standing in air at room temperature (percent) | Elongation of the sample after shrinking treatment for 12 min. in 100° C. water free of tension (percent) |
| Control 2              | 100                      | 20                         | 62          | 1.75             | 221                  | 0.06                                                | 25                                   | 34                                                                      | 450                                                                                                       |
| Control 3              | 140                      | 15                         | 49          | 1.91             | 165                  | 0.08                                                | 38                                   | 26                                                                      | 405                                                                                                       |
| Example 2              | 160                      | 8                          | 44          | 2.41             | 110                  | 0.11                                                | 54                                   | 15                                                                      | 388                                                                                                       |
| Example 3              | 180                      | 5                          | 41          | 2.88             | 103                  | 0.12                                                | 55                                   | 8                                                                       | 370                                                                                                       |
| Example 4              | 190                      | 3                          | 42          | 2.73             | 107                  | 0.11                                                | 53                                   | 9                                                                       | 375                                                                                                       |

#### Control

For comparison, the drying was insufficiently performed leaving 3.0 wt. percent of the solvent in the same filaments which were subsequently drawn, heat set, cooled and shrunk in the same manner as above. The properties of the resultant spandex filaments are given in Table 2. As can be seen, the control filaments failed to show the high elasticity of the spandex filaments of this invention,

70 Thus with the heat setting temperature of below 150° C., sufficient heat setting effect cannot be obtained. Of course at the temperature below 150° C. still satisfactory result could be obtained with prolonged setting time if the drawing temperature is also below 150° C., but such is not industrially recommendable. Particularly, when the spinning step is immediately followed by high speed processing, such prolonged treatment is not practical from the point of equipments.

Accordingly the heat setting temperature should be no lower than 150° C. in order to perform the heat setting of the invention with good efficiency.

## EXAMPLE 5

A polyurethane elastic polymer synthesized by reacting polycaprolactam having a molecular weight of 1,700 and terminal hydroxyl radicals with 4,4'-diphenylmethane diisocyanate and ethylene glycol at the molar ratio of 1.0:5.0:4.0 was thoroughly dried, drawn, heat set, cooled and shrunk in the similar manner as described in Example 1. Thus prepared spandex filaments (40 deniers) showed a tenacity of 2.71 g./d., an elongation of 98% and a shrinkage in 100° C. water of 52%. When the same was further shrunk under the same shrinking conditions employed in Example 1, its elongation increased to 366%. On the other hand, filaments similarly prepared from a polyurethane elastic polymer obtained by reacting a prepolymer of polytetramethylene glycol having a molecular weight of 2,180 and 4,4'-diphenylmethane diisocyanate with ethylene diamine as the chain extender failed to exhibit sufficient low elongation set effect.

## EXAMPLE 6

A dimethylformamide spinning solution (28% concentration) of a polyurethane elastic polymer obtained by reacting the following three components, i.e., polyethylene butylene adipate having a molecular weight of 1950 and terminal hydroxyl radicals (ethylene:butylene copolymerization ratio=8:2), 2,6-tolylene diisocyanate and 1,4-butanediol, mixed at the molar ratio of 1.5:4.5:4.0 was dry-spun into a spinning column similar to that employed in Example 1, and thereby spun filaments having a remaining dimethylformamide content of 4.5 wt. percent were obtained. After standing in a room of 20° C. for 10 hours, the filaments were dried on Nelson rollers of 175° C. driven at a rate of 300 m./min. for 8 seconds to have a reduced dimethylformamide content of 0.37 wt. percent. Thereafter the filaments were drawn by 4 times between two rollers heated to 135° C., heat set on heat-setting rollers of 180° C. which were driven at a rate of 1200 m./min. for 6 seconds, cooled to about 22-23° C. on cooling rollers of 20° C. driven at a rate of 1200 m./min. for 3 seconds, and shrunk by 10% as they were taken up onto a take-up roller of 20° C. driven at a rate of 1080 m./min. Thus obtained spandex filaments having a denier of 38 had a tenacity of 2.60 g./d. and an elongation of 80%. Whereas the same filaments, after the subsequent treatment in 100° C. water for 12 minutes free of tension, had a tenacity of 1.13 g./d. and an elongation of 390%, thus returning to the conventional spandex filaments of low tenacity and high elongation as they were before the treatments of the subject invention.

In contrast, the spandex filaments prepared under exactly same conditions to the above except that the 1,4-butanediol as the chain extender was replaced by hydrazine showed at 40 deniers a tenacity of 1.73 g./d. and an elongation of 340%, thus showing no low elongation set effect.

## EXAMPLE 7

A dimethylacetamide spinning solution (32% concentration) of a polyurethane elastic polymer obtained by mixing and reacting the three components of polyethylene butylene adipate having a molecular weight of 1950 and terminal hydroxyl radicals (ethylene:butylene copolymerization ratio=8:2), 4,4'-diphenylmethane diisocyanate and ethylene glycol at a molar ratio of 1.0:5.0:4.0, was dry-spun into a spinning column similar to that employed in Example 1, and whereby spun filaments having a remaining dimethylacetamide content of 3.3 wt. percent were obtained. Continuously to the spinning step, the filaments were dried on Nelson rollers heated to 175° C. and driven at a rate of 330 m./min. for 5 seconds, to be given a reduced dimethylacetamide content of 0.33 wt.

percent. Then the filaments were drawn by 3 times between two rollers heated to 145° C., heat set on heat setting rollers of 185° C. driven at a rate of 990 m./min. for 7 seconds, cooled on cooling rollers of 25° C. driven at a rate of 990 m./min. for 5 seconds, and further shrunk by 5% as they were taken up onto take-up rollers of 20° C. driven at a rate of 940 m./min. Thus obtained spandex filaments had a denier of 35 and an elongation of 101%. When the same was further subjected to a shrinking treatment for 10 minutes in 100° C. water free of tension, the filaments showed an elongation of 415%, thus exhibiting excellent elastic recovery.

## EXAMPLE 8

A spinning solution of 30% concentration was prepared by dissolving the powdery polyurethane elastic polymer of Example 1 in dimethylacetamide instead of dimethylformamide. The same was subsequently spun under the same conditions employed in Example 1 and continuously thereafter dried for 7 seconds on Nelson rollers at 180° C. The dimethylacetamide content of the resultant filaments was, to the filaments, 0.41% by weight. The filaments were thereafter treated under the same drawing, heat setting, cooling and shrinking conditions as of Example 1, giving spandex filaments of low elongation (elongation of 40 denier spandex filaments=87%), high tenacity (2.70 g./d.) and high Young's modulus (tenacity at 10% elongation=0.2 g./d.).

When the same spandex filaments were treated in 100° C. water for 8 minutes free of tension, its elongation became 410%. Thus the product showed an excellent low elongation set effect.

For comparison, the above procedures were repeated except that the spun filaments still containing 0.75 wt. percent of dimethylacetamide were treated, yielding spandex filaments of which elongation was 115%. The same filaments, after 8 minutes' treatment in 100° C. water free of tension, had an elongation of 283%, thus failing to regain the elongation of 413% possessed before the drawing.

We claim:

1. Process for the continuous preparation of spandex filaments having a temporarily lowered elongation of less than 120% and a tenacity of 2.0-4.0 g./den., characterized in that a spinning solution of a polyurethane elastic polymer prepared from a polymer diol having a molecular weight of 500-5,000, an aromatic diisocyanate and a diol having a molecular weight of 50-200, dissolved in an organic solvent of boiling point below 200° C. is dry spun and the resulting filaments are subjected to treatments comprising, in succession:
  - (1) drying the spun filaments at a temperature above the boiling point of the solvent but no higher than 200° C. to reduce the residual solvent content to no more than 0.5% by weight,
  - (2) drawing the filaments to 2-6 times their original length at a temperature of 80-150° C.,
  - (3) heat setting the drawn filaments at a temperature of 160-200° C.,
  - (4) cooling the heat set filaments to a temperature below 50° C.,
  - (5) causing the filaments to shrink by 5-15% of their original length.
2. The process for the continuous preparation of temporarily low elongation set spandex filaments according to claim 1, in which the low molecular diol is ethylene glycol.
3. The process for the continuous preparation of temporarily low elongation set spandex filaments according to claim 1, in which the polyurethane elastic polymer is that obtained by the reaction of polyethylene propylene adipate having a molecular weight of 500-5,000, 4,4'-diphenylmethane diisocyanate, and ethylene glycol.
4. The process according to claim 1, in which the solvent is selected from a group consisting of dimethyl-

3,476,850

9

formamide, dimethylacetamide, tetrahydrofuran and di-methylsulfoxide.

References Cited

UNITED STATES PATENTS

2,755,266 7/1956 Brenschede ----- 260—32.6  
2,956,330 10/1960 Pitzl ----- 264—290  
2,957,852 10/1960 Frankenburg et al. --- 260—75  
3,227,972 1/1966 Rosenthal et al. ----- 264—203  
3,353,344 11/1967 Clendening ----- 57—34

10

FOREIGN PATENTS

916,287 1/1963 Great Britain.

DONALD J. ARNOLD, Primary Examiner

H. MINTZ, Assistant Examiner

U.S. CL. X.R.

28—72; 57—168; 264—210, 235, 342, 290